

Nov. 3, 1925.

1,560,201

J. BINGHAM

MANUFACTURE OF SHEET METAL ARTICLES

Filed Nov. 3, 1924



Inventor

Jeremiah Bingham,

By Anna Ann Crayton

Attorney

## UNITED STATES PATENT OFFICE.

JEREMIAH BINGHAM, OF TOLEDO, OHIO, ASSIGNOR TO THE AMERICAN-NATIONAL COMPANY, OF TOLEDO, OHIO, A CORPORATION OF OHIO.

## MANUFACTURE OF SHEET-METAL ARTICLES.

Application filed November 3, 1924. Serial No. 747,410.

To all whom it may concern:

Be it known that I, JEREMIAH BINGHAM, a citizen of the United States, and a resident of Toledo, in the county of Lucas and State of Ohio, have invented a new and useful Manufacture of Sheet-Metal Articles, which invention is fully set forth in the following specification.

This invention relates to sheet metal articles, and particularly to the manufacture of articles of this class of light gage metal, having elongated rolled portions which are given small radius bends transversely of their axes.

In the manufacture of sheet metal articles, it is desirable in many cases to form the articles with edge rolls both to provide a finished edge and to give strength and rigidity to the article, and in some cases to provide a hand grip on the article. Where the edge of the article is straight the roll of the edge may be made of any diameter, but if it is desired to transversely bend the roll in a small radius to cause it to conform to the shape of the edge of the article, as for instance the body wall of a juvenile vehicle wagon, it is extremely difficult to accomplish this particularly where the metal is of light gage, as in such wagon bodies without injury to the roll by reason of buckling the roll at the inner side of the bend or breaking the metal of the roll at the outer side of the bend.

It has been found to be a comparatively simple proposition to bend metal pipes without damaging or distorting the metal and this has been accomplished, in some instances, by the use of coil-springs which are inserted inside the pipes in the region of the bend. In some instances these springs have been allowed to remain in the pipes, but generally they are removed after the pipes are bent. A much more difficult problem, however, is presented in the bending of sheet metal strips having rolled edges, because, instead of working on a circumferentially unbroken structure, a longitudinally elongate slit is provided which materially increases the difficulty in bending the metal without distortion. Numerous methods have been attempted for accomplishing this result but, so far as I am aware, no one has ever before successfully

bent sheet metal strips having rolled edges without in some way injuring the roll. 55

The primary object of this invention is to so reinforce a sheet metal roll of any diameter, within reason, as to enable it to be transversely bent without flattening, buckling or breaking. 60

While the invention in its broader aspect is capable of being practiced in numerous ways, a preferred method of practicing same is illustrated in the accompanying drawings, in which,— 65

Fig. 1 is a perspective view of a strip of sheet metal having its longitudinal edges formed with straight rolls with reinforcing or form-maintaining means embodying the invention disposed within the rolls, portions of the metal being broken away; and Fig. 2 is an edge view thereof with a strip and its rolls transversely bent at the point of reinforcement and with portions broken away. 75

Referring to the drawings, 1 designates a strip of sheet metal having, in the present instance, each of its longitudinal edges formed with a roll 2. It will be understood, however, that the number of rolls used or the location of the same whether at the edges of the strip or intermediate such edges is immaterial, so far as the invention is concerned, so long as the roll is so disposed that it is bent transversely of its axis 85 in the forming of the article for which the strip is used.

It is evident that if a roll 2, the diameter of which is greater than approximately  $\frac{1}{4}$  of an inch, were bent or given a curve transversely of its axis, as shown in Fig. 2, the roll would either be flattened in the bending action, or it would be buckled at the inner side of its bend or broken at its outer side due to the stresses set up by the bending action, and usually a breaking of the roll at its outer side occurs. The use of a wire in the roll would be objectionable in many cases for the reason that it could not be removed from the roll after the bending 95 operation, and would, therefore, add considerable weight to the article.

My invention contemplates the use in the roll during the bending action of a form-maintaining member which will prevent collapsing of the roll and which, at the same 105

time, is sufficiently yielding or pliable in its nature to allow it to accommodate itself to the movement of the metal in the bending operation. For this purpose I employ a 5 form-maintaining slug or member 3 of a relatively softer material than the sheet metal, such, for instance, as lead, and introduce it in the roll throughout the length of the portion thereof to be bent. This form- 10 maintaining member is of a cross-sectional size sufficient to substantially fill the hollow of the roll and may be introduced into the roll during the forming of the same, or after it has been formed, as may be desired. 15 During the transverse bending of the sheet metal and roll, the member 3 is bent therewith and prevents collapsing of the roll and at the same time the yielding nature thereof permits it to accommodate 20 itself to the different portions of the metal of the roll during the bending thereof and consequent stretching of the metal of the roll, and breaking of the roll is thereby prevented. In other words, the soft metal 25 or material forming the member 3 moves in accordance with the movement of the contacting portions of the metal roll during

the bending operation, and thereby effect- 30 tually prevents breaking or other injury to the roll while being bent.

After the sheet metal piece and roll have been bent in the desired form, heat is applied to the roll to effect a melting and flowing of the material of the member 3 from the interior of the roll. 35

Having thus described my invention, what I claim as new and desire to secure by Letters Patent is:

1. The method of bending a sheet metal blank which consists in providing a blank with an edge roll, inserting into the roll a core of metal softer than the metal of the blank, transversely bending the blank with the roll and core, and heating the roll to melt and thereby remove the core. 40
2. The method of bending a sheet metal blank which consists in providing a blank with an edge roll, inserting a lead core into the roll, transversely bending the blank with the roll and core, and heating the roll to melt the core thereby to remove the core. 45

In testimony whereof I have hereunto signed my name to this specification.

JEREMIAH BINGHAM.